

## UNITED STATES PATENT OFFICE.

HERBERT COFFMAN, OF SAN MATEO, CALIFORNIA.

## SMUDGING AND FROST-PREVENTING COMPOSITION.

No Drawing.

Application filed August 16, 1922. Serial No. 582,298.

*To all whom it may concern:*

Be it known that I, HERBERT COFFMAN, a citizen of the United States of America, residing at San Mateo, in the county of San Mateo and State of California, have invented certain new and useful Improvements in Smudging and Frost-Preventing Compositions, of which the following is a specification.

10 This invention relates to compositions of matter and has special reference to a solid fuel compound.

More particularly the invention relates to the composition of a solid fuel for smudging 15 and frost prevention.

It is common, at present, to protect the trees in orchards in the early spring from the blighting by frost, especially when the trees are in bloom or early fruitage, by raising the temperature of the atmosphere in such an orchard by building fires at intervals between the trees. Under the present methods these fires, usually using oil as a fuel, are built in special burners or stoves.

25 This method is objectionable for various reasons among which may be mentioned the expense of the burners, as one of these special devices is ordinarily used for every four trees; and the work required to place 30 and feed these burners since they must be moved out of the way to enable the ground between the trees to be cultivated and replaced each night to be ready for sudden frosts in the morning.

35 The principal object of the present invention is the provision of an improved solid composition fuel especially adapted for smudging and frost preventing and which may be burnt directly on the ground without any special burners or other draft producing devices being necessary.

40 A second important object of the invention is the provision of improved fuel of this class which may either be used in bulk 45 or in briquetted form.

A third important object of the invention is the provision of such an improved fuel which may be readily lit and which will burn freely notwithstanding its position directly on the ground.

With the above and other objects in view, as will be hereinafter apparent, the invention consists of an improved fuel composition hereinafter fully described and 55 specifically claimed.

In the formation of this composition I

preferably employ as one of the principal ingredients, carbon in a more or less pure form and it has been found that the oil-gas residue, known as lamp black, which is a by-product obtained in the manufacture of illuminating gas from crude oil, is one of the best forms of carbon to use although charcoal or lignite may also be employed. In any event it has been found advisable to 60 grind the carbon used to a powder. To a suitable quantity of the carbon is added a quantity of saw dust of the same weight, the sawdust being employed just as it comes from the mill, in which condition it may or may 65 not contain a certain proportion of shavings or small chips. To these two are added a quantity of crude oil equal in weight to the combined weights of the carbon and saw dust, the mass being slightly heated to facilitate absorption of the oil. Finally, in order 70 to promote and hasten the combustion of the fuel, there is added to the mass approximately 20% of its total weight of sodium nitrate. These ingredients are thoroughly 75 blended by stirring or mixing in some suitable mechanical mixing device.

The fuel thus prepared can be shipped in bulk or packed in suitable containers such as paper bags or the like and can be distributed in the packages or in heaps between the trees.

It has also been found that the quantity of crude oil may be slightly reduced and pitch or asphaltum added to form a better 80 binder so that the composition may be pressed into suitable briquettes. To do this, it is preferred to employ from 5 to 7½% of the pitch or asphaltum, properly heated. These briquettes are preferably perforated 85 to increase combustion.

The composition thus formed has the 90 property of burning at first with a high intensity, this continuing until the more volatile elements have been consumed, after 95 which it will continue to burn with practically no flame until practically all of the composition has been burnt, there being very little ash left. This gives the fuel a high 100 value for its purpose since the temperature is quickly raised above the danger point by the quick first burning and is kept there by the slower final burning. Further, it is 105 peculiarly adapted to the small grower of apricots or prunes in particular as the localities in which these fruits are grown 110 are seldom subjected to danger from frost.

more than once or twice a year and thus an expensive outlay for stoves or burners of very little use is avoided.

Having thus described the invention, what 5 is claimed as new, is:—

1. As a new composition of matter, a solid fuel for smudging and frost prevention including in combination ground carbon, sawdust, crude oil, and sodium nitrate in proportions suitable to produce smoke and heat and ensure complete combustion of all ingredients.
- 10 2. As a new composition of matter, a solid fuel for smudging and frost prevention including in combination, that oil gas residue called lamp black in a finely ground condition, sawdust, crude oil and sodium nitrate in proportions suitable to produce smoke and heat and ensure complete combustion of
- 15 3. As a new composition of matter, a solid

fuel for smudging and frost prevention comprising in combination equal parts of that oil gas residue called lamp black in a finely ground condition, and sawdust, crude oil 25 substantially equal in weight to the lamp black and sawdust, and sodium nitrate in an amount equal to 20% of the weight of lamp black, sawdust and crude oil.

4. As a new composition of matter, a solid fuel for smudging and frost prevention comprising in combination equal parts of that oil gas residue called lamp black in a finely ground condition, and sawdust, crude oil 30 substantially equal in weight to the lamp black and sawdust, sodium nitrate in an amount equal to 20% of the weight of lamp black, sawdust and crude oil, and substantially 5% of pitch like substance.

In testimony whereof I affix my signature.

HERBERT COFFMAN.